

Jan. 28, 1941.

T. L. DUNBAR

2,229,886

## METHOD OF DIGESTING FIBROUS MATERIALS

Filed Dec. 19, 1934

2 Sheets-Sheet 1



Inventor  
THOMAS L. DUNBAR

Raymond J. Norton  
Attorney

Jan. 28, 1941.

T. L. DUNBAR

2,229,886

METHOD OF DIGESTING FIBROUS MATERIALS

Filed Dec. 19, 1934

2 Sheets-Sheet 2

FIG. 3.



Inventor  
THOMAS L. DUNBAR

Raymond J. Norton  
Attorney

## UNITED STATES PATENT OFFICE

2,229,886

## METHOD OF DIGESTING FIBROUS MATERIALS

Thomas L. Dunbar, Watertown, N. Y., assignor to Chemipulp Process Inc., Watertown, N. Y., a corporation of New York

Application December 19, 1934, Serial No. 753,314

10 Claims. (Cl. 92—7)

This invention relates to an improved method of and apparatus for the digestion of fibrous material.

In the usual method of digesting wood chips by the quick cook method the digester is first completely filled with chips and then acid is admitted. The mass is brought up to reaction temperatures by admitting direct steam. Ordinarily the steam is admitted slowly for it had been thought that this was necessary to permit the liquor to penetrate the chips and thus to insure thorough cooking of the centers of the chips. Thus, under the old practice, from about two to four hours were allowed for this preliminary saturation period, that is to say the admission of steam was controlled so that a temperature of approximately 110°—170° C. was reached only after the two to five hour period.

In the early stages of the cook the chips settled and during subsequent cooking the relief was so manipulated that the chips were completely immersed in the liquor. This was thought to be necessary for it was believed that exposed or uncovered chips would be over cooked or burned.

Recently, as disclosed in the U. S. patent to Dunbar 1,859,384, it has been proposed to first saturate the chips with hot acid under high hydrostatic pressure prior to the actual commencement of the cook and in this way to more quickly initiate the boiling and to economize on steam consumption.

It has now been found that if the chips are subjected to a thorough saturation with the reagent employed for digestion and the pressure and liquid level then properly adjusted prior to cooking, an improved process resulting in a better quality and higher yield of pulp is obtained. The preliminary saturating treatment is specially correlated with regard to pressure and temperature conditions during the cook so that as a result it is possible to effect the cook with a greatly diminished quantity of the reagent and with a quantity less than that necessary to completely submerge the chips. While no definite statement of the mechanism of the reaction is advanced, it would appear that at least a portion of the fibrous material is digested in a vapor or a mixed liquid-vapor phase rather than in a continuous liquid phase as heretofore.

It is therefore an object of the present invention to provide a new method of delignifying cellulosic material.

Another object is to provide a novel digestion

process characterized by a markedly reduced liquor requirement.

Another object is to devise a process of digesting pulp in which cellulose losses are minimized.

A further object is to provide a process of the character described in which heating costs are materially diminished.

With these and other equally important and related objects in view, the invention comprehends the concept of subjecting fibrous material such as wood chips to a special preliminary treatment whereby the chips are thoroughly saturated with a digestion reagent and subsequently cooking such chips under improved conditions of pressure concentration and quantity of reagent.

In order more clearly to explain the invention there is shown in the accompanying drawings a typical form of apparatus which may be employed to effectuate the process, in which:

Figure 1 is an elevation of one form of apparatus, certain well known parts being omitted for simplicity.

Fig. 2 is a detail of the digester illustrating the relationship of chip and liquor levels.

Fig. 3 is a diagram of temperature and pressure conditions obtaining during typical treatments according to the invention.

In the past it was generally assumed that an essential condition of digestion of chips was a complete submergence of the chips in the digesting liquor, for it was found that when the liquid level was lowered below the level of the chips a considerable degree of burning of the uncovered chips occurred. In the older methods, such burning almost of necessity occurred for the chips were wetted with acid only on the surface or to a small depth below the surface. Under the thermal conditions of the older operations such surface liquid was evaporated. Since the liquid medium, in effect, served as the thermal control, such relatively dry chips were overcooked.

I have found that a digestion process may be carried out in which a high liquid level need not be maintained if certain conditions are fulfilled. Such conditions essentially are a complete saturation of the chips with the digestion agent at temperatures below but preferably close to reaction temperatures and such a control of the conditions of temperature and pressure that the upper portion of the mass of chips is in contact with the reagent in the vapor or mixed liquid and vapor phase.

5 Thorough impregnation of the chips is rather difficult to achieve. The chips themselves are a heterogeneous substance: the fibrous structure contains substances which are of differential chemical compositions, hardness, porosity and permeability. Thus the structural composition of the middle lamella differs from that of the secondary layers of the cell wall. It is therefore difficult to force a saturating solution 10 into the chips so as to insure a substantially uniform penetration coupled with uniform concentration of the saturant throughout the body of the chip.

15 When, however, such thorough and homogeneous saturation has been effected the material then becomes a potentially reactive mass, presenting an optimum surface of contact of the main reactive materials, i. e. the acid (or equivalent reagent) and the ligno-cellulose aggregates. By reason of this physical condition a 20 novel type of digestion is possible.

25 The conditions to be observed in impregnating the chips to secure the thorough saturation will vary somewhat depending upon the particular type of raw material and reagent employed. Due to the great complexity, from a chemical and physicochemical standpoint, of the fibrous material treated, it is extremely difficult to positively define the mechanism of the reaction. However, 30 it does appear that such impregnation does involve such phenomena as selective solubility, osmosis, the ionic condition of the saturant, and possibly cataphoresis. Of these, selective solubility and osmosis undoubtedly play a very important 35 part. The hot acid, employed in the present process for the saturant, takes into solution certain of the non-cellulosic and non-ligneous material, such for example as some of the polysaccharides other than cellulose. The acid also 40 mixes with the water held in the prosenchymatous elements of the wood. As is known, there may be a considerable variation in this water, mechanically held for the most part, and known as the moisture content. It is quite probable that 45 the mechanism of impregnation is quite analogous to the phenomena involved in the normal vital processes of the plant and presents the same type of selectivity of passage or permeability, permitting relatively pure substances like water to 50 permeate the membranes quite freely, ionic solutions like dissolved salts less readily, and complex organic substances least of all. Hence the characteristics of the impregnating solution, such as its temperature and hydrogen ion concentration, are important features to be taken into 55 consideration.

60 In carrying out the present process hot acid (below reaction temperatures) is employed as a saturant and this is employed under conditions of excess quantity of acid, high hydrostatic or penetrating pressure and optimum recirculation. Due to the relatively high temperatures employed the acid tends to penetrate the cellular structure more rapidly. The recirculation tends not 65 only to a uniform temperature throughout the mass, that is to say of both the acid and the chips, but also serves to leach or wash out some of the acid soluble and mechanically held substances in the wood. When the wood is treated under these 70 conditions of a hot, high pressure, recirculating acid for a sufficient period of time, depending upon the particular impregnant and the raw material treated, a thorough saturation of the fibrous material may be obtained.

75 In these circumstances a digestive reagent,

namely the acid, at a uniform and relatively high temperature, is practically homogeneously distributed through the mass and held in the inter- and intra-cellular spaces. This type of preliminary treatment therefore is carefully to be distinguished from other forms of initial treatments in which the woody structure is merely wetted on the surface. A chip which is thoroughly saturated, in the manner described, tends to retain the liquid content under much more drastic conditions of temperature than would a surface wetted chip. It is believed that the novel digestion process of the present invention, involving a low liquid level, is permitted by this fact.

80 In the second stage of the improved process, 15 that is the digestion stage proper, the conditions are so regulated that a low liquid level is maintained, that is to say a liquid level below the level of the chips even after the chips have settled to their maximum degree. In these circumstances it is probable that a portion of the chips are actually digested in a mixed liquid and vapor phase. Due to the effective preliminary saturation the digesting liquor is held within the body of the chips and is there raised to reaction temperatures. Due to the optimum surface contacts, coupled with the initial elevated temperature of the acid, the mass may be quickly brought into reaction. During digestion a relatively high partial pressure of gas is maintained in the digesting 30 zone so as to commensurately inhibit the evolution of free SO<sub>2</sub> from the liquid medium; in other words to maintain the free acid concentration of the liquor.

35 Another important feature of the present invention made possible by the thorough preliminary impregnation is that the mass is quickly brought up to reaction temperatures. In the preferred method of operation this is achieved by rapidly diminishing the pressure after the saturating period so that a maximum quantity of steam, and hence of heat units, may be admitted at the commencement of the cook. The preliminary saturating period therefore eliminates the necessity heretofore obtaining in the art of bringing up the steam pressure slowly.

40 The principles of the invention will more readily be appreciated upon a consideration of a specific illustrative process in which they are embodied.

45 As shown in the drawings, a unit may comprise as the major apparatus elements the acid storage tank 1, the hot acid accumulator 2 and any desired number of digesters 3. Where the digestive reagent is a metal bisulphite this may be admitted 50 to the storage tank from the acid towers by means of the pump 4 and line 5. Such acid is usually at relatively low temperature. If desired this acid may be given a mild degree of preheat either by interposing a heat exchange in line 4 or a closed 55 heating coil in the tank. When the acid in tank 1 is at atmospheric pressure the temperature cannot be greatly raised without loss of SO<sub>2</sub> gas. The liquid in tank 1 is also preheated by hot overhead accumulator gas vented through line 6 60 and relatively low pressure digester gases entering through line 7 in a manner more fully to be described.

65 The accumulator 2, which is preferably spherical in shape, serves a number of important purposes in the present method. It is of relatively great capacity and functions as a heat regenerative plant in which heat units of the hot fluids discharged from the digester are imparted to a body of cooler acid admitted from the storage 70

75

5 tank; coincidentally such cooler acid absorbs free gas evolved during the cooking. The accumulator is so constructed and designed that the temperature, pressure and concentration of the acid may 5 carefully be controlled within narrow ranges. This is of especial importance in the present method which, as noted above, involves an optimum temperature of the acid during the penetration period.

10 For these several purposes therefore the accumulator is in communication with the acid storage tank 1 through the pump 8, line 9, drop leg 11, second eductor 12 and discharge branch 13. The eductor 10 is connected to the relief header 14 associated with the digester. The line 9 is 15 preferably provided with the check valve 9'. The eductors are each provided with suitable control valves 10' and 12' respectively whereby the flow of fluids therethrough may be regulated.

20 It will be seen that relatively cool (or slightly preheated) digester liquor may be forced under any desired velocity by pump 8 through line 9 and eductor 10, thence through the drop leg 11 and eductor 12 to the accumulator. Eductor 10, 25 being in communication with line 14, aspirates fluids in the line and thus induces a suction or diminished pressure, depending in degree upon the particular construction of the eductor and the velocity of the acid flowing through line 9. The 30 condensable or absorbable components of this fluid are condensed by and/or absorbed in the flowing stream of cooler acid. Such double action is accentuated and supplemented by the second eductor 12 in the same fluid line.

35 The second eductor 12, as shown, is connected in a separate accumulator recirculation circuit. This comprises the drawoff or inlet branch 15, controlled by valve 15', recirculating pump 16 and discharge line 17. When pump 16 is operated 40 liquor is withdrawn from the accumulator and forced, at any desired velocity, through line 17 to intimately contact with fluids flowing into the eductor 12 through the drop leg 11. In order more accurately to control the temperature of 45 the acid within the accumulator either a direct or indirect heater may be interposed at any desired point in the recirculating line.

50 Where the exigencies of a particular situation so recommend, the eductor 12 may be omitted and the drop leg 11 may be connected to the suction side of pump 16, the line 17 then being directly connected to the accumulator. While the lines 13 and 15, for simplicity, are shown closely 55 spaced near the bottom of the accumulator, it will of course be understood that they may be located at any desired position. Thus the draw-off line may be positioned near the bottom and the discharge line 13 at any desired elevation. An advantage of placing the line 15 near the 60 bottom is that the induced circulation in the accumulator is then contra to the natural (convective) flow and thus tends to a more uniform temperature throughout the mass of liquid.

65 As noted above, the pressure conditions within the accumulator may be controlled within any desired range. To accomplish this the vent line 6 is provided with a pressure regulating valve 6' so that whenever the pressure in the accumulator rises above a determined point, say of the order 70 of from twenty-five to one hundred pounds more or less, gases are automatically vented to the storage tank 1. Similarly a bypass line 18 provided with a pressure regulating valve 18' leads from the header 14 to the top of the accumulator. 75 This valve may be set at any desired pressure

differential, say of the order of from one to three or four pounds. When the pressure in relief line 14 exceeds by this amount the pressure in the accumulator, the valve 18' operates and fluids are bypassed around the eductor and passed directly 5 to the accumulator.

The accumulator is provided with the gauge glass 19 to indicate the liquid level and this enables the operator to control the flow of fluids thereto. A liquid level indicating and/or recording instrument may also be utilized.

One or, as shown, a battery of digesters may be employed. These are each provided with a removable manhole cover to permit charging of the chips. The relief branch 21, provided with control valve 21', leads from the upper portion of the digester to the main header 14. A second relief line 22, provided with the control valve 22', leads from the upper section of the digester to the low pressure header 7, through which low pressure 20 gases are vented to the storage tank or other absorber. The line 22 is provided with a branch 23, controlled by valve 23', which may discharge to the atmosphere. The side relief line 24, having the control valve 24', leads from a relatively 25 low point of the digester to the header 14. It will be noted that when this side relief line is opened the liquid level in the digester may be brought to a low point which is materially below the normal level of the chips. The gauge glass 30 25 is lengthened to extend a suitable distance below the liquid level which obtains during the cooking operation.

The digesters may be charged with acid from the accumulator through the line 26, valve 26', pump 27, header 28 and inlet branches 29. These branches may selectively be connected to the header by properly manipulating the valves 29' in the manner well known.

35 In accordance with principles hereinbefore explained, the digester is provided with means to recirculate the liquor during the saturating stage and when desired during any desired period of the cooking stage. For this purpose the recirculating line 30 is provided with the inlet branches 40 45 31 and 32 which extend within the digester and are suitably perforated. The branches are provided with the control valves 31' and 32' respectively so that one or both can be connected to line 30. The other end of line 30 is connected to 50 the suction side of pump 33 and this discharges through line 34 into the lower portion of the digester.

55 In one preferred modification a heater 35 is provided in the recirculation circuit, the purpose of which is to maintain the recirculating stream of acid at the optimum temperature during the soaking period. Consonant with this purpose the flow of heating medium through the heater may be controlled by a thermostatic 60 element so positioned as to be responsive to the temperature of the liquor in the circuit and preferably to that within the digester. The heater 35 may be of any desired type, such as an indirect heat exchange, the heating medium of which may be steam, hot spent liquor, waste gases or the like.

65 Since the present invention permits the use of a relatively strong acid during the soaking period, and since such soaking is carried out at elevated 70 temperatures, means are provided to maintain the acid concentration and conserve heat units by returning any evolved gas to the soaking liquor. As shown, a gas line 37 leads from the upper portion of the digester and discharges into the liquid recirculation line preferably through 75

the eductor 38. It will be understood that any free gas which is liberated from the liquor during the soaking period may thus be returned to maintain the free acid concentration of the soaking liquor as well as to conserve the heat value in the gas.

If desired such gas line 37 may also be employed as a means of increasing the free acid concentration. Thus, if desired, the line 37 may be connected by a valved branch to header 14 so that the aspirating effect of the eductor 38 will be applied to the fluid in header 14. Hence, whenever desirable, hot relief fluids discharged from a mass of chips undergoing digesting may be admitted to another mass of chips undergoing soaking, preferably in the manner indicated, that is into the recirculating stream by way of an eductor. Heat is thus directly imparted to the soaking liquor and the free acid content of such liquor raised. It will thus be seen that the temperature of the soaking liquor may be controlled by direct heat exchange with hot fluids and/or by indirect methods, as by the heater 35. By proper regulation of these two the temperature and concentration of the acid may be maintained at any desired value.

The concentration of the liquor in the digester, both during the soaking period and the subsequent digestion period, may, if desired, automatically be controlled by utilizing a tank of liquid or gaseous  $\text{SO}_2$  and controlling the flow of this gas into the digester by means of an electric controller, such for example as shown in prior Patent 1,888,632. Such control is well known in the art and may comprise essentially a pair of plates or electrodes, the current through which is a function of the concentration of the liquor (electrolyte). This type of electrical control may also be employed to govern the flow of relief fluids from the header into the digester recirculating line during the soaking period.

The temperature required to be developed for the actual cooking of the chips may be derived from any suitable source. In the preferred method the temperature is brought up by means of direct steam admitted from a steam header through a plurality of steam inlets 40.

The digesters are provided with suitable temperature and pressure recording instruments by means of which a continuous record of these two factors, plotted against time, as indicated in Fig. 3, may be obtained. The digesters are also provided with valved blow off lines (not shown) through which pulp is discharged at the end of the cook.

The character of the process of digestion will have been appreciated from the foregoing description of the apparatus. It may be assumed that material within say the second digester is undergoing digestion and relief fluids are flowing through header 14 and valves 21', 22' and 24' of number one digester are closed. In starting the treatment in the first digester the manhole cover 20 is removed and the digester completely filled with chips. The cover is then bolted and valves 21', 22' and 24' are kept closed and valve 23' is opened. Valves 26' and 29' are then opened and hot acid from accumulator 2 is admitted to the first digester. Since a relatively high pressure obtains in the accumulator, hot acid rapidly flows into the digester. Upon diminution of this flow the pump 27 may be started to force the acid into the digester. As acid enters the digester the air contained therein is displaced and escapes

through open valve 23'. When  $\text{SO}_2$  gas or liquor begins to discharge from line 23 the valve 23' is closed and the pump 27 maintained in operation until a high hydrostatic pressure is built up on the acid.

When the acid has been pumped in so as to obtain a high pressure, of the order of seventy to ninety or more pounds, the valves 26' and 29' are closed and pump 27 stopped. Valves 21', 22' and 24' are maintained closed and valve 31' (and if desired valve 32') is opened. The pump 33 is then operated and the high pressure acid is withdrawn from the upper and forced into the lower part of the digester.

In Fig. 3 there are shown graphically two typical runs utilizing the present process; the full lines indicating the temperature and pressure condition in one and the broken lines indicating these conditions of the other. As shown in Fig. 3, the hot acid admitted from the accumulator soon reaches a practically constant value of about 75° C. or 80° C. in the illustrative methods. During its passage through the recirculation circuit heat may be imparted to the acid by means of the heat exchange 35 so as to compensate for that absorbed by the chips. As noted above, the degree of heat imparted to the recirculating acid may automatically be controlled so as to establish and maintain the temperature of the acid at any predetermined value. The action of the heater 35 may be supplemented by means of the introduction of hot relief fluids conveyed from header 14 to line 37 by a branch line (not shown) or by the introduction of direct steam from a line (not shown).

During this recirculation any gases evolved from the liquor in the digester are withdrawn through line 37, mixed with and absorbed in the hot recycle liquor in eductor 38 and returned to the digester. The insertion of the eductor 38 in the recycle line serves to impose a reduced pressure in line 37 and thus facilitates the withdrawal of gases. When the line 37 is connected to header 14 the eductor functions similarly.

The time of recirculation may vary considerably depending upon such factors as the character of the chips, temperature of the acid, etc. In the illustrated procedures, starting with relatively warm acid, the recirculation may be continued for approximately one and one-half hours (as shown in the full lines), or about four hours (as shown in dotted lines). During this time, using apparatus of typical size, the equivalent of approximately three or more digester charges of acid is recirculated through the chips.

Such recirculation, as noted, displaces air from the digester, preheats and saturates the chips with hot acid close to reaction temperature, and leaches and removes the "extractives" from the chips. Optimum penetration and area of contact is thus achieved.

It is particularly to be observed that while the preliminary impregnation is by recirculation to and from the digester, the process is not limited to this. Thus the major advantage may be secured by including the accumulator in such recirculation circuit. In such circumstances hot acid may be forced by pump 27 through the digester, thence through a line extending from branch 31 or 32 to the accumulator 2. In such an operation the heater corresponding to heater 35 and an eductor corresponding to eductor 38 may be interposed in line 28 and the drop leg 37 connected to this line.

After the chips have been thoroughly saturated the conditions within the digester are then adjusted rapidly to bring the mass up to reaction temperatures. For this purpose the pressure is 5 materially dropped (as shown in Fig. 3) and heat units imparted. After the soaking period therefore the recirculating pump 35 is stopped and liquor is relieved from the digester through the side relief 24 until, as shown in Fig. 2, the level 10 (B) of the liquor is well below the level (A) of the chip. In these circumstances there is, as shown on the chart, a decided and abrupt drop in pressure from the order of eighty-five or ninety pounds down to thirty pounds more or less. This, 15 as will be appreciated, enables the employment of low pressure direct steam for bringing the mass up to reaction temperature. Such relief flows through header 14, eductor 10 and drop leg 11 into the accumulator.

20 While at first blush it would appear that such a drastic drop in pressure would seriously dilute the acid, due to evaporation of  $\text{SO}_2$ , such loss does not in fact obtain to any material degree. This would appear to be due to the fact that a 25 large volume of the acid is actually held in the inter- and intra-cellular spaces of the chips and hence the free surface of the acid is much less than would be expectable from that quantity of acid. Furthermore, during the latter stages of 30 such withdrawal, i. e. when the pressure is lower and a commensurate increase in the evolution of  $\text{SO}_2$  would be expected, a large quantity of the gas is constrained to pass through a mass of wetted chips which tend to reabsorb and probably 35 to adsorb the gas.

As indicated above, the preferred heating medium is direct steam introduced through the steam inlets 40. As shown on the chart, admission of the steam soon builds up the pressure 40 within the digester and the temperature then increases at a relatively rapid rate. After the pressure has been raised to the operating level, this may then be maintained by opening valve 21'. In order to insure uniform thermal conditions 45 during the beginning, or any later stage, of the reaction, the liquid may be recycled to and from the digester by closing the branch 31, opening the branch 32 and pumping the liquor through the recirculating line. By operating the heater 35 50 during this recycling period the quantity of direct steam and extent of condensation and consequent dilution of acid can correspondingly be controlled.

During the progress of the cook the liquid level 55 tends to raise due to the increased volume of condensate. As shown in Fig. 3, the top relief 21 may be closed and side relief 24 opened and liquor withdrawn some time after reaction temperatures have been reached, and in the illustrated methods after the fourth and sixth hours 60 respectively. By proper manipulation of valves 21' and 24' the desired low liquid level may be maintained.

During this period a relatively large quantity 65 of chips is above the liquid level and is undergoing digestion. Since these exposed chips are thoroughly saturated into the core the reaction proceeds when reaction temperatures are reached. Such chips therefore may be considered as being 70 contacted with liquid acid on the interior and on the external surfaces with a mixed liquid and vapor phase of the reagent. In any event, whatever may be the mechanism of the reaction, it is found that with the described low liquid 75 level treatment the uncovered chips are uniform-

ly and thoroughly digested and produce the same character of pulp as that immersed in the liquor.

As is known in the art, as the reaction proceeds a considerable quantity of free gas is evolved. This is probably due to the fact that the reaction produces organic acids which tend to displace and set free an equivalent amount of sulphurous acid. This tends to build up an excess pressure. In the present operation such pressure is relieved by opening valve 21' and recovering the chemical and heat values by absorbing such gases in the eductor 10, drop leg 11 and eductor 12. In typical operations according to the present method such gas relief may be operated a short time after the fifth hour in one case and after the sixth hour in the other. This relief is controlled, as shown in Fig. 3, so as to maintain the pressure substantially constant down to the blow down period. In the present method pressures during the cooking are maintained at approximately seventy-five pounds and optimum temperature of about 135° C.

It is to be observed that in one form of the present process the maximum reacting temperature is reached at about the eighth hour in one case and the seventh hour in another, and this may be maintained at a substantially constant pressure, by proper manipulation of the valves, until the usual tests indicate the approximate termination of the cook. Steam is shut off some time prior to completion of the cook, in the manner known to those skilled in the art. The pressure is reduced gradually down to 20 or 30 lbs., after which the material is either discharged into the blow-pit or is washed with water and then discharged.

It will be seen that the present type of process presents many advantages. As will be observed from an inspection of the chart, the preliminary saturation period is carried out under high pressure and in such circumstances as to insure a substantially uniform and relatively high temperature of the mass prior to the cooking period. The quantity of heat units therefore required are materially diminished inasmuch as there is much less of a temperature rise required than in prior processes. As compared, for example, to a cold acid cook, the heat units necessary are only those required to bring the mass from a temperature of 70° or 80° up to cooking temperatures (of the order of 115° C.) as against a rise from 40° to 100° C. This diminishes the steam consumption and the liquor necessary to be withdrawn on side relief.

As noted hereinbefore, the preliminary treatment insures a thorough saturation of the chips with acid at a uniform temperature and a uniform concentration. As a result of this type of treatment marked economies are secured. Thus, according to the older methods of digestion, using small size digesters, about 2500 gallons of liquor were required per ton of pulp. When utilizing the principles of the present invention, with the same size digester, the quantity of liquor can be reduced to between 1800 and 2000 gallons. 65 This results not only in large savings in handling costs but also in sulphur and steam costs, the steam cost being reduced substantially in direct proportion to the reduction in the quantity of liquor required. Furthermore, due to the thorough impregnation, a larger ultimate yield is secured because this type of treatment reduces the quantity of shives or uncooked cores in the final product.

The process is so operated as to insure op-

timum recovery of the heat units as well as the chemical values of the liquor.

An outstanding feature of the present invention resides in the fact that it permits the use of a low liquid level without in any way impairing the quality of the pulp produced. The lowering of the liquid level, permitted by the special preliminary treatment, as noted above, effects savings in the quantity of liquor required and establishes corresponding economies in chemical and steam costs. It will be understood that while the type of recirculation shown is from the top to the bottom of the digester, such recirculation may, by the proper by-pass connections to the pump, be made from the bottom to the top, so that if desired during a single soaking and/or cooking period recirculation may be from top to bottom, bottom to top, or an intermittent use of these two.

Therefore, while a preferred modification of the invention has been described, it is to be understood that this is given merely to exemplify the underlying principles involved. It will be readily apparent to those skilled in the art that these salient principles may be effectuated in other specifically different types of methods and one utilizing different apparatus. Thus, while a process has been described with respect to the digestion of wood chips with bi-sulphite liquor, it is apparent that it is applicable to other digestion processes operating upon different raw materials and utilizing different reagents. Similarly, while a process has been described with respect to the quick cooking method, i. e. use of direct steam as the heating medium, it is clear, as has been pointed out, that the mass may be brought to reaction temperatures by using indirect heating methods or by a combination of the two. Therefore the invention is not to be considered limited to the particular procedures described, except as such limitations are clearly imposed by the appended claims.

I claim:

1. In the digestion of fibrous material in which the material is submitted to a soaking with hot digestion liquor below reaction temperature prior to cooking, that improvement which comprises pumping the hot liquor continuously and directly to and from the digester during such soaking operation and utilizing such pumping operation for simultaneously withdrawing gases from the digester and returning such gases in admixture with liquor to the digester.

2. In a process of the character described, charging a digester with fibrous material, storing hot preconditioned acid in an accumulator, charging hot acid from the accumulator to the digester and then circulating the hot liquor to and from the digester while maintaining the liquor below reaction temperature, the utilizing the recirculating stream to withdraw gas from the gas space of and return it to the body of liquid in the digester.

3. In a process of the character described, admitting a charge of fibrous material to be delignified to an enlarged digestion chamber, accumulating hot preconditioned digestion liquor in a separate tank, pumping hot liquor from the tank to the digester until a high hydrostatic pressure is established, then pumping the liquor directly to and from the digester for a period of time sufficiently prolonger to insure substantially complete penetration of the material, and subsequently lowering the liquid level in the digester 75 to a point below the level of the material and

then raising the liquor to reaction temperatures.

4. A process of digesting fibrous material which comprises admitting the material to an enlarged digester, introducing digester liquor at elevated but below reaction temperature to the digester, utilizing such liquor to displace and vent air from the digester, sealing the digester from access of air while admitting an additional quantity of hot liquor sufficient in amount to establish a high hydrostatic pressure on the acid, then recirculating the acid directly to and from the digester for a relatively protracted period while maintaining it below reaction temperature, then drawing off liquor from the digester to a degree to expose at least a portion of the material before raising the mass to reaction temperature.

5. A method of digesting fibrous materials which comprises admitting the material to an enlarged chamber to completely fill the chamber, introducing preheated bisulphite liquor maintained at temperatures above 60° C. but below reaction temperatures, building up a high hydrostatic pressure on the liquor and recirculating it to and from the digester, maintaining the optimum temperature of the liquor during such recirculation by applying heat thereto, continuing such circulating until a uniform temperature is attained and the material is subsequently completely impregnated with the hot liquor; then lowering the liquid level well below the level of the material and bringing the mass up to reaction temperatures and during such reaction maintaining a high partial pressure of acid gas in the vapor space of the chamber.

6. A method of digesting fibrous materials which comprises filling a digester with the material, admitting hot digestion liquor to the digester while displacing and venting air therefrom, sealing the digester against access of air and admitting additional quantities of the hot bisulphite liquor to impose a high hydrostatic pressure thereon, then recirculating the hot acid directly to and from the digester while automatically regulating the temperature to an optimum value which accelerates penetration but precludes any substantial reaction; maintaining all the material in contact with the acid for a period of time sufficiently prolonged to insure optimum penetration, then withdrawing a sufficient quantity of the liquor to establish a large vapor space in the digester and expose a considerable quantity of the chips above the liquid level, and then bringing the mass up to digestion temperatures while maintaining a high partial pressure of sulphur dioxide gas in the vapor space.

7. A method of digesting fibrous material which comprises charging the material to a digester, admitting hot digester liquor below reaction temperature to the digester and contacting it with the material for a period sufficiently long to insure penetration of the liquor into the material while recirculating the liquor to and from the digester, withdrawing relief fluids from a second mass of material undergoing digestion and admitting such fluids to the said mass undergoing penetration to control the temperature and concentration of said soaking liquor, withdrawing liquor from the digester and lowering the liquid level to a point materially below the level of the material and cooking such material in hotter digestion liquor.

8. In the digestion of fibrous materials in which the material is submitted to soaking with hot digestion liquor maintained at elevated but be- 75

low reaction temperatures prior to cooking, that improvement which comprises forcing a quantity of hot digestion liquor maintained below reaction temperatures into a digester until a high hydrostatic pressure has been established on the liquor, pumping the liquor directly to and from the digester while maintaining the liquor below a temperature at which any substantial cooking takes place, and utilizing such pumping operation for simultaneously withdrawing gases from the upper portion of the digester and returning such gases in admixture with liquor back into the digester.

9. A process of digesting fibrous material which comprises admitting the material to an enlarged digester, introducing a charge of hot digestion liquor to the digester, such charge being greater than that required to fill the digester at normal pressure, the temperature of the liquor being below reaction temperature; recirculating the liquor directly to and from the digester, heating the liquor during such recirculation to maintain it at an elevated optimum but below reaction temperature, continuing such recircula-

tion until the material has been penetrated with liquor, then materially lowering the liquid level below the level of the material in the digester and cooking the mass.

10. A method of digesting fibrous material which comprises filling a digester with the material, admitting hot digestion liquor to the digester while displacing and venting air therefrom, sealing the digester against access of air and admitting additional quantities of the hot liquor to impose a high hydrostatic pressure thereon; then recirculating the hot acid to and from the digester while automatically regulating the temperature and concentration to an optimum value which accelerates penetration but precludes any substantial reaction; maintaining all of the material in contact with the liquor for a period of time sufficiently prolonged to insure optimum penetration, then withdrawing a sufficient quantity of the liquor to establish a vapor space in the digester and expose a considerable quantity of the chips above the liquid level, and then bringing the mass up to digestion temperatures.

THOMAS L. DUNBAR.